# EUROPEAN PATENT SPECIFICATION

(11) **EP 0 309 158 B1**
(45) Date of publication and mention of the grant of the patent: **10.02.1993**
(21) Application number: 88308567.2
(22) Date of filing: 16.09.1988
(51) Int. Cl.: G03C 7/26, G03C 7/38

(54) **Photographic recording material comprising a magenta dye image forming coupler compound**
Photographisches Eintragungsmaterial mit einer ein purpurrotes Farbbild bildenden Kupplerverbindung
Matériau photographique d'enregistrement comprenant un composé copulant formant une image de couleur magenta

(30) Priority: 21.09.1987 US 99171
(43) Date of publication of application: 29.03.1989
(73) Proprietor: EASTMAN KODAK COMPANY (a New Jersey corporation), Rochester, New York 14650 (US)
(72) Inventor: Merkel, Paul Barrett c/o EASTMAN KODAK COMPANY, Rochester New York 14650 (US)
(74) Representative: Baron, Paul Alexander Clifford

(56) References cited:
- EP-A- 0 232 624
- EP-A- 0 268 496
- DE-A- 3 226 163
- PATENT ABSTRACTS OF JAPAN, vol. 9, no. 72 (P-345)[1795], 2nd April 1985

## Description

This invention relates to a color photographic silver halide recording material. In particular, the invention relates to an improved photographic recording material containing a magenta dye image-forming coupler compound.

Color photographic recording materials generaly contain silver halide emulsion layers sensitized to each of the blue, green and red regions of the visible spectrum, with each layer having associated therewith a color-forming compound which, respectively, yields a yellow, magenta or cyan dye. The quality of the resulting color image is primarily based on the dye hues obtained from the respective color-forming compounds.

Magenta dye image-forming couplers are frequently employed to provide desired magenta dye images. A problem encountered with such couplers is that the spectral absorption characteristics of dyes obtained therefrom may not have the particular absorption maximum and distribution that are desired. Frequently, a dye which is obtained may have an absorption maximum as little as several nanometers removed from the optimum desired value, and therefore will not have the desired hue, notwithstanding this slight difference in absorption characteristics. Conversely, a resulting dye may have an absorption maximum which is considerably shorter than a desired value.

Attempts to alter absorption characteristics of dyes, including those obtained from magenta dye image-forming coupler compounds, are usually focused on alterations of the structures of coupler compounds. This approach, while enjoying some measure of success, is time consuming and involves the expense of highly focused research programs. Success with such research is not predictable so that improvements in final hue values have been elusive even after concentrated research efforts.

Some coupler solvents are known to cause shifts in absorption values of dyes. For example, U.S. Patent 3,676,137 describes use of a phosphate ester of a high boiling coupler solvent to shift absorption of a cyan dye to a shorter wavelength in order to reduce excessive red wavelength absorption. Alternatively, Japanese Patent Publication No. 59(1984) - 102234 describes the use of high boiling phenolic compounds to shift the spectral absorption of 2,5-diacylaminophenol cyan dye-forming coupler compounds to longer wavelengths. However, as is shown below by comparative data, a phenolic compound of this publication does not provide a sufficient level of hue shifting as compared with that obtained with the present invention.

Japanese Patent Publication No. 59(1984) - 204041 describes use of urea compounds with cyan dye image-forming couplers to improve light fastness, to reduce unwanted green absorption and to reduce loss of density caused by bleach operations in dyes obtained from such couplers. This publication also suggests addition of other compounds that form dyes by oxidative coupling with primary amine color developing agents, such as magenta and yellow coupler compounds. However, there is no teaching or suggestion in this publication that particular urea compounds can be used to alter absorption characteristics of dyes derived from magenta dye forming coupler compounds.

Accordingly, the object of the present invention is to provide a color photographic silver halide recording material having the capability of imparting slight as well as relatively large alterations in absorption properties of a magenta dye to obtain a spectral absorption value different from the inherent absorption characteristics of the dye.

This object is achieved with a color photographic recording material which comprises a support having thereon a light-sensitive silver halide emulsion layer, a magenta dye image-forming coupler capable of forming a dye by reaction with oxidized color developing agent and, associated with the coupler, a urea compound which is capable of altering the spectral absorption of the magenta dye formed from the coupler, said urea compound having the structural formula: wherein;
R¹ is a substituted or unsubstituted alkyl or an aryl group having from 6 to 12 carbon atoms which may be substituted with halogen, alkoxy or carboalkoxy groups having from 2 to 12 carbon atoms, or alkyl having from 1 to 20 carbon atoms; R² is hydrogen or a substituted or unsubstituted alkyl group;
R³ is a substituted or unsubstituted alkyl or alkoxy group having from 1 to 20 carbon atoms or an electron-withdrawing group which is -CN, -N0₂, a halogen atom, -COR⁴ or S0₂R⁴, wherein R⁴ is an alkyl or an alkoxy group having from 1 to 20 carbon atoms or an aryl or an aryloxy group having from 6 to 12 carbon atoms, and
n is from 0 to 3;

This invention also relates to a color photographic record comprising a magenta dye formed by a coupling reaction between a magenta dye image-forming coupler and oxidized silver halide developing agent, which recording material comprises, in association with the dye, a urea compound having the structural formula: wherein;
R¹ is a substituted or unsubstituted alkyl or an aryl group having from 6 to 12 carbon atoms which may be substituted with halogen, alkoxy or carboalkoxy groups having from 2 to 12 carbon atoms, or alkyl having from 1 to 12 carbon atoms;
R² is hydrogen or a substituted or unsubstituted alkyl group;
R³ is a substituted or unsubstituted alkyl or alkoxy group having from 1 to 20 carbon atoms or an electron-withdrawing group which is -CN, -N0₂, a halogen atom, -COR⁴ or S0₂R⁴, wherein R⁴ is an alkyl or an alkoxy group having from 1 to 20 carbon atoms or an aryl or an aryloxy group having from 6 to 12 carbon atoms, and
n is from 0 to 3;
R¹ can be represented by alkyl groups having from 1 to about 20 carbon atoms, preferably from 1 to about 12 carbon atoms, which groups can be straight or branched chain and optionally can be substituted. Aryl groups which can be represented by R¹ have from about 6 to about 12 carbon atoms, which groups are optionally substituted.
Useful R² groups are hydrogen or alkyl as defined for R^{1.}

The most preferred urea compounds are those where R¹ is an alkyl group having from about 4 to about 10 carbon atoms and where R² is hydrogen.

R³ substituents can be alkyl or alkoxy groups having from 1 to about 20 carbon atoms, preferably from 1 to about 12 carbon atoms, which groups can be straight or branched chain and which can be substituted.

Substituents which can be present on the R¹ and R² groups include halogen atoms, such as chlorine and bromine, and alkoxy or carboalkoxy groups wherein the total number of carbon atoms in such groups is from 2 to about 12. When R¹ is aryl the substituents can also be alkyl, preferably alkyl having from 1 to about 12 carbon atoms.

Electron-withdrawing groups represented by R³ include -CN, -N0₂, a halogen atom, and -S0_{2R}⁴,

where R⁴ is an alkyl or an alkoxy group having from 1 to about 20 carbon atoms or an aryl or an aryloxy group having from about 6 to about 12 carbon atoms.

Chlorine is a preferred halogen substituent on the phenyl group inasmuch as it provides good stability properties and is least expensive to manufacture.

The described urea compounds can be easily synthesized in quantitative yield by adding amines to isocyanates according to the procedures known in the art. Two or more urea compounds may be used in combination to alter the spectral absorption properties of magenta dyes as described herein.

There are no particular restrictions on the quantity of a urea compound which can be employed with a magenta dye image-forming compound either alone or in combination with known coupler solvents. Generally, it is desirable that the quantity of urea compound, with respect to each part by weight of the magenta coupler, be from 0.05 to 10 parts, preferably from 0.2 to 3 parts by weight of the coupler compound. As the amount of urea compound increases, relative to the amount of magenta coupler compound employed, there is usually a detectable increase in the extent of hue shift in the magenta dye. However, the particular choice of magenta coupler, of urea compound or the presence of one or more coupler solvents, all tend to influence the type and the extent of spectral absorption change in the resulting magenta dye.

When the magenta coupler compound is added to a silver halide emulsion, conventional procedures may be employed. For example, the coupler can first be dissolved in one or more known coupler solvents, such as di-n-butyl phthalate (DBP), and then be mixed with a urea compound as described herein. If desired, the magenta coupler compound can be mixed with a urea compound where these compounds are sufficiently compatible so that known coupler solvents may not be needed. The resulting mixture or solution is then dispersed in aqueous gelatin, preferably containing a surfactant, and the dispersion is added to a silver halide emulsion which can then be coated by known techniques.

Specific urea compounds which are useful for shifting the absorption values of magenta dyes obtained from the reaction of magenta dye-forming couplers with oxidized color developing agent include the following:

Couplers which form magenta dyes upon reaction with oxidized color developing agents are described in such representative patents and publications as: U.S. Patent Nos. 1,969,479; 2,311,082; 2,343,703; 2,369,489; 2,600,788; 2,908,573; 3,061,432; 3,062,653; 3,152,896; 3,519,429; 3,725,067; 4,443,536; European Patent Publication 170164; European Patent Publication Nos. 177,765; and copending U. S. Patent Applications Ser. No. 23,517 of S. Normandin et al, filed March 9, 1987; Ser. No. 23,518 of R. Romanet et al, filed March 9, 1987; No. 23,519 of A. Bowne et al, filed March 9, 1987 and Ser. No. 23,520 of A. Bowne et al, filed March 9, 1987.

Preferred magenta couplers include pyrazolones having the structural formulae: and pyrazolotriazoles having the structural formulae: or pyrazolobenzimidazoles having the structural formulae: and and indazoles having the structural formula: wherein
R⁶ is halogen (e.g., chloro, fluoro), alkyl or alkoxy having from 1 to 4 carbon atoms, phenyl or substituted phenyl (e.g., 2,4,6-trihalophenyl);
R⁷ is a ballast group;
R⁸ is hydrogen or a monovalent organic radical, for example a saturated or unsaturated alkyl group having from 1 to about 20 carbon atoms (methyl, ethyl, propyl, butyl, decyl, dodecyl, heptadecyl, octadecyl); a cycloalkyl group (e.g. cyclohexyl); an aralkyl group (e.g. benzyl); an aryl group (e.g. phenyl, alkylphenyl or alkoxyphenyl in which the alkyl or alkoxy radical has from 1 to about 20 carbon atoms, nitrophenyl, aminophenyl, acylaminophenyl, alkyl- aminophenyl, naphthyl, diphenyl, diphenylether, diphenyl- thioether); a heterocyclic group (e.g. a-furyl, a-benzofuryl, q-pyridyl); an amino, hydroxy or carboxylic acid group, it being possible for the hydrogen atoms of these groups to be substituted, for instance by a mono-or dialkylamino group in which the alkyl groups have from 1 to about 20 carbon atoms; a cycloalkylamino group; an amino group in which one hydrogen atom is replaced by a pyrazolo-[1,5-a]-benzimidazolyl radical which is bonded in 3- position to said nitrogen atom so that couplers result in which two pyrazolo-[1,5-a]-benzimidazolyl radicals are connected by an amino group, and in which the remaining hydrogen atom may be replaced by a substituent such as an alkyl-, aryl-, aralkyl- or acyl- radical; an acylamino group in which the acyl radical is derived from an aliphatic, aromatic or heterocyclic carboxylic acid; a carboxylic acid group which is esterified by means of an aliphatic, cycloaliphatic or aromatic alcohol or by an aromatic compound having a phenolic hydroxy group; or a carboxyamido group in which the amido group may be substituted for example by a saturated or unsaturated alkyl, aralkyl, aryl or heterocyclic group;
R⁹ represents a hydrogen atom, a sulphonic acid or a carboxylic group; a halogen atom (e.g. chlorine or bromine); or an azo radical -N = NR¹⁴, wherein R14 can be an aromatic or heterocyclic radical (phenyl, naphthyl, diphenyl, diphenylether, benzthiazolyl, pyridyl, quinolyl or pyrazolyl) which may be substituted such as by an alkyl group having from 1 to about 20 carbon atoms, hydroxy, alkoxy, halogen, amino, substituted amino, nitro, sulphonic acid or carboxylic acid groups;
R¹⁰ represents a divalent radical such as wherein R¹¹ can be alkyl, aralkyl, especially phenyl, phenyl substituted preferably in the p-position by a tertiary amino group such as a dialkylamino group in which at least one of the alkyl groups is substituted by carboxy, sulpho, hydroxy, alkoxy, carboxylalkyl, cyano or the divalent radical wherein R¹² and R¹³ represent aliphatic, aromatic, araliphatic or heterocyclic radicals, and
X represents hydrogen or a coupling off group.

Specific magenta dye forming coupler compounds which are useful in the practice of this invention include:

Photographic elements in which the photographic couplers of this invention are incorporated can be simple elements comprising a support and a single silver halide emulsion layer, or they can be multilayer, multicolor elements. The coupler compounds of this invention can be incorporated in the silver halide emulsion layer or in another layer, such as an adjacent layer, where they will come into reactive association with oxidized color developing agent which has developed silver halide in the emulsion layer. The silver halide emulsion layer can contain, or have associated therewith, other photographic coupler compounds, such as color forming couplers, colored masking couplers, etc. These other photographic coupler compounds can form dyes of the same or different color and hue as the photographic coupler compounds of this invention. Additionally, the silver halide emulsion layer can contain addenda conventionally contained in such layers.

A typical multilayer, multicolor photographic element according to this invention comprises a support having thereon a red-sensitive silver halide emulsion layer having associated therewith a cyan dye image-forming coupler compound, a green-sensitive silver halide emulsion layer having associated therewith a magenta dye image-forming coupler compound and a blue-sensitive silver halide emulsion layer having associated therewith a yellow dye image-forming coupler compound, wherein the magenta dye image-forming coupler compound has associated therewith a urea compound as described herein. Each silver halide emulsion layer can be composed of one or more layers and the layers can be arranged in different locations with respect to one another. Typical arrangements are described in U.S. Patent Nos. 3,227,554; 3,620,747; 3,843,369; and 4,400,463 and in U.K. Patent No. 923,045.

The light sensitive silver halide emulsions can include coarse, regular or fine grain silver halide crystals or mixtures thereof and can be comprised of such silver halides as silver chloride, silver bromide, silver bromoiodide, silver chlorobromide, silver chloroiodide, silver chlorobromoiodide and mixtures thereof. The emulsions can be negative-working or direct-positive emulsions. They can form latent images predominantly on the surface of the silver halide grains or predominantly on the interior of the silver halide grains. They can be chemically and spectrally sensitized. The emulsions typically will be gelatin emulsions although other hydrophilic colloids can be used in accordance with usual practice.

The support can be of any suitable material used with photographic elements. Typically, a flexible support is employed, such as a polymeric film or paper support. Such supports include cellulose nitrate, cellulose acetate, polyvinylacetal, polyethylene terephthalate, polycarbonate and resinous materials as well as glass, paper or metal. Paper supports can be acetylated or coated with baryta and/or an a-olefin polymer, particularly a polymer of an a-olefin containing 2 to 10 carbon atoms such as polyethylene, polypropylene or ethylene-butene copolymers.

Further details regarding silver halide emulsions and elements, and addenda incorporated therein can be found in Research Disclosure, December 1971, Item 9232, Paragraphs I through XVIII. Research Disclosure is published by Industrial Opportunities Ltd., Homewell, Havant, Hampshire, P09 1 EF, United Kingdom.

The term "in association" is intended to mean that materials can be in either the same or different layers, so long as the materials are accessible to one another.

The following examples further illustrate the invention. Unless otherwise indicated all parts, percents and ratios are by weight.

### Example 1

Single layer coatings containing silver bromoiodide emulsion (6.5 mole % I) comprising unsensitized polydisperse medium-large grains (0.91 gAg/m²) were prepared on cellulose acetate-butyrate supports. Each layer also contained gelatin (3.8 g/m²) and the magenta coupler C-4 (1.3 g/m²) as described above. The coupler was dispersed in di-n-butyl phthalate (DBP) (1.3 g/m² when used alone) or in combination of DBP and a urea compound (each at 0.65 g/m²) as described below in Table 1. Each coating was exposed imagewise through a graduated-density test object to provide a maximum density image and was processed at 33 C employing the color developer solution described below, and then subjected to 1.5 minutes in the bleach-fix bath described below, washed and dried.

Transmission density versus wavelength data were obtained to determine the λ-max of the dye in an environment with the addition of different dispersants. The data show a desirable and noticeable shift in hue to longer wavelength with addition of urea compounds.

As can be seen from the data in Table I, hue shifts are highly subtle and vary only a few nanometers from the control. Such variations in wavelength shifts offer a high degree of manipulative control and provide an excellent, inexpensive means to obtain particularly desired hue values.

### Example 2

This example is similar to Example 1, except that pyrazolotriazole magenta coupler C-14 (1.3 g/m²) as described above, was used:
Coatings were prepared, exposed, processed, and evaluated as in Example 1. The same color developing agent and DBP (di-n-butyl phthalate) coupler solvent were used. Resulting data are reported in the following Table:

### Example 3

In another evaluation, not involving coupling to form a dye within a silver halide emulsion photographic system, the hue shifting of preformed magenta dyes was examined. A dye, a urea compound as described in Table III and the coupler solvent DBP (di-n-butyl phthalate) were mixed, dispersed in a gelatin vehicle and then coated in a single layer.

Evaluations of transmission density vs wavelength data were obtained and are reported in Table III.

Dye structures: As can be seen from Table III the described urea compounds are capable of shifting magenta dye hue to longer wavelengths.

Inasmuch as the dyes utilized in Table III were all preformed and therefore avoided conventional aqueous processing, it can be appreciated that the concept of altering the spectral absorption of dyes is applicable to other than conventional photographic systems.

## Claims

1. A color photographic recording material comprising a support having thereon a light-sensitive silver halide emulsion layer, a magenta dye image-Forming coupler capable of forming a dye by reaction with oxidized color developing agent and, associated with the coupler, a urea compound which is capable of altering the spectral absorption of the magenta dye formed from the coupler, said urea compound having the structural formula: wherein;
R¹ is a substituted or unsubstituted alkyl or an aryl group having from 6 to 12 carbon atoms which may be substituted with halogen, alkoxy or carboalkoxy groups having from 2 to 12 carbon atoms, or alkyl having from 1 to 12 carbon atoms;
R² is hydrogen or a substituted or unsubstituted alkyl group;
R³ is an unsubstituted or a substituted alkyl or alkoxy group having from 1 to 20 carbon atoms or an electron-withdrawing group which is -CN, -N0₂, a halogen atom, -COR⁴ or S0₂R⁴, wherein R⁴ is an alkyl or an alkoxy group having from 1 to 20 carbon atoms or an aryl or an aryloxy group having from 6 to 12 carbon atoms, and
n is from 0 to 3.

2. A photographic recording material according to claim 1 wherein R³ is chloro.

3. A photographic recording material according to any of claims 1 or 2 wherein R⁴ is an alkyl group having from 1 to 12 carbon atoms.

4. A photographic recording material according to any of claims 1 to 3 wherein R¹ is an alkyl group having from 1 to 20 carbon atoms or an aryl group having from 6 to 12 carbon atoms.

5. A photographic recording material according to any of claims 1 to 4 wherein R² is an alkyl group having from 1 to 20 carbon atoms.

6. A photographic recording material according to any of claims 1 to 5 wherein R¹ is an alkyl group having from 4 to 10 carbon atoms and R² is hydrogen.

7. A photographic recording material according to any of claims 1 to 6 wherein the magenta dye image-forming coupler is a pyrazolone, pyrazolotriazole, pyrazolobenzimidazole or indazole compound.

8. A photographic recording material according to any of claims 1 to 7 wherein the urea compound is present in an amount of from 0.05 to 10, preferably from 0.2 to 3 parts by weight of coupler compound.

9. A photographic recording material according to claim 1, 7 or 8 wherein the urea compound has one of the structural formulae: or or or

10. A color photographic record comprising a magenta dye Formed by a coupling reaction between a magenta dye image-Forming coupler and oxidized silver halide developing agent, which recording material comprises, in association with the dye, a urea compound as defined in any of claims 1 to 9.

## Patentansprüche

1. Farbphotographisches Aufzeichnungsmaterial mit einem Träger, auf dem sich befinden eine lichtempfindliche Silberhalogenidemulsionsschicht, ein ein purpurrotes Farbstoffbild liefernder Kuppler, der einen Farbstoff durch Umsetzung mit oxidierter Farbentwicklerverbindung zu erzeugen vermag und eine dem Kuppler zugeordnete Harnstoffverbindung, welche die spektrale Absorption des aus dem Kuppler gebildeten Purpurrotfarbstoffes zu verändern vermag, wobei die Harnstoffverbindung der folgenden Strukturformel entspricht: worin bedeuten:
R¹ eine substituierte oder unsubstituierte Alkylgruppe oder Arylgruppe mit 6 bis 12 Kohlenstoffatomen, die gegebenenfalls durch Halogen, Alkoxy-oder Carbalkoxygruppen mit 2 bis 12 Kohlenstoffatomen substituiert sein kann oder durch Alkyl mit 1 bis 12 Kohlenstoffatomen;
R² Wasserstoff oder eine substituierte oder unsubstituierte Alkylgruppe;
R³ eine unsubstituierte oder substituierte Alkyl- oder Alkoxygruppe mit 1 bis 20 Kohlenstoffatomen oder eine elektronenabziehende Gruppe bestehend aus -CN, -N0₂, einem Halogenatom, -COR⁴ oder -S0₂R⁴, worin R⁴ für eine Alkyl- oder Alkoxygruppe mit 1 bis 20 Kohlenstoffatomen steht oder eine Aryl- oder eine Aryloxygruppe mit 6 bis 12 Kohlenstoffatomen, und
n gleich 0 bis 3.

2. Photographisches Aufzeichnungsmaterial nach Anspruch 1, worin R³ für Chlor steht.

3. Photographisches Aufzeichnungsmaterial nach einem der Ansprüche 1 oder 2, worin R⁴ eine Alkylgruppe mit 1 bis 12 Kohlenstoffatomen ist.

4. Photographisches Aufzeichnungsmaterial nach einem der Ansprüche 1 bis 3, worin R¹ eine Alkylgruppe mit 1 bis 20 Kohlenstoffatomen darstellt oder eine Arylgruppe mit 6 bis 12 Kohlenstoffatomen.

5. Photographisches Aufzeichnungsmaterial nach einem der Ansprüche 1 bis 4, worin R² eine Alkylgruppe mit 1 bis 20 Kohlenstoffatomen ist.

6. Photographisches Aufzeichnungsmaterial nach einem der Ansprüche 1 bis 5, worin R¹ eine Alkylgruppe mit 4 bis 10 Kohlenstoffatomen ist, und R² für Wasserstoff steht.

7. Photographisches Aufzeichnungsmaterial nach einem der Ansprüche 1 bis 6, worin der ein purpurrotes Farbstoffbild liefernde Kuppler eine Pyrazolon-, Pyrazolotriazol-, Pyrazolobenzimidazol- oder Indazolverbindung ist.

8. Photographisches Aufzeichnungsmaterial nach einem der Ansprüche 1 bis 7, worin die Harnstoffverbindung in einer Konzentration von 0,05 bis 10, vorzugsweise von 0,2 bis 3 Gewichtsteilen Kupplerverbindung vorliegt.

9. Photographisches Aufzeichnungsmaterial nach Anspruch 1, 7 oder 8, worin die Harnstoffverbindung eine der folgenden Strukturformeln aufweist: oder oder oder

10. Farbphotographische Aufzeichnung mit einem purpurroten Farbstoff, der durch Kupplungsreaktion zwischen einem ein purpurrotes Farbstoffbild liefernden Kuppler und oxidierter Silberhalogenidentwicklerverbindung erzeugt worden ist, wobei das Aufzeichnungsmaterial in Verbindung mit dem Farbstoff eine Harnstoffverbindung nach einem der Ansprüche 1 bis 9 enthält.

## Revendications

1. Produit d'enregistrement photographique en couleurs comprenant un support portant une couche d'émulsion aux halogènures d'argent sensible à la lumière, un coupleur formateur d'image de colorant magenta capable de former un colorant par réaction avec le développateur chromogène oxydé et, associé avec le coupleur, un composé urée qui est capable d'altérer le spectre d'absorption du colorant magenta formé à partir du coupleur, le composé urée ayant la structure: où
R¹ est un groupe aryle ou alkyle substitué ou non ayant de 6 à 12 atomes de carbone qui peut être substitué avec des groupes halogènes, alkoxy ou carboalkoxy ayant de 2 à 12 atomes de carbone, ou un groupe alkyle ayant de 1 à 12 atomes de carbone ;
R² est un atome d'hydrogène ou un groupe alkyle substitué ou non ;
R³ est un groupe alkoxy ou alkyle substitué ou non ayant de 1 à 20 atomes de carbone ou un groupe attracteur d'électrons qui est -CN, -N0₂, un atome d'halogène, -COR⁴ ou S0₂R⁴, où R⁴ est un groupe alkoxy ou alkyle ayant de 1 à 20 atomes de carbone ou un groupe aryloxy ou aryl ayant de 6 à 12 atomes de carbone, et
n est compris entre 0 et 3.

2. Produit d'enregistrement photographique selon la revendication 1 dans lequel R³ est un groupe chloro.

3. Produit d'enregistrement photographique selon l'une quelconque des revendications 1 ou 2 dans lequel R⁴eSt un groupe alkyle ayant de 1 à 12 atomes de carbone.

4. Produit d'enregistrement photographique selon l'une quelconque des revendications 1 à 3 dans lequel R¹ est un groupe alkyle ayant de 1 à 20 atomes de carbone ou un groupe aryle ayant de 6 à 12 atomes de carbone.

5. Produit d'enregistrement photographique selon l'une quelconque des revendications 1 à 4 dans lequel R² est un groupe alkyle ayant de 1 à 20 atomes de carbone.

6. Produit d'enregistrement photographique selon l'une quelconque des revendications 1 à 5 dans lequel R¹ est un groupe alkyle ayant de 4 à 10 atomes de carbone et R² est un atome d'hydrogène.

7. Produit d'enregistrement photographique selon l'une quelconque des revendications 1 à 6 dans lequel le coupleur formateur d'image de colorant magenta est un composé pyrazolone, pyrazolotriazole, pyrazolobenzimidazole ou indazole.

8. Produit d'enregistrement photographique selon l'une quelconque des revendications 1 à 7 dans lequel la quantité du composé urée est comprise entre 0,05 et 10, de préférence, entre 0,2 et 3 parties en poids de coupleur.

9. Produit d'enregistrement photographique selon la revendication 1,7 ou 8 dans lequel le composé urée à la formule : ou ou

10. Enregistrement photographique en couleurs comprenant un colorant magenta formé par réaction de couplage entre un coupleur formateur d'image de colorant magenta et un développateur d'halogénures d'argent oxydé, un tel produit d'enregistrement comprend, en association avec le colorant, un composé urée selon l'une quelconque des revendications 1 à 9.
